

## UNITED STATES PATENT OFFICE.

HENRY R. POWER, OF NIAGARA FALLS, NEW YORK, ASSIGNOR TO THE CARBORUNDUM COMPANY, OF NIAGARA FALLS, NEW YORK, A CORPORATION OF PENNSYLVANIA.

## ABRASIVE COMPOSITION.

No Drawing.

Application filed May 31, 1922. Serial No. 564,959.

My invention relates to abrasive compositions for grinding metal surfaces, such as valve seats for internal combustion engines, although the composition may be used for 5 any grinding operation where a tight joint is desired between the two metal surfaces.

The present grinding compositions for such purposes are of two classes, one class comprising the abrasive grains mixed with 10 grease or oil. On account of the lubricating action of the grease or oil, the full cutting value of the abrasive grains is not obtained in this class. In the second class, the abrasive grains are mixed with water 15 and an organic binder such as gum, starch, lichen or seaweed. The objection to this class is that on drying, a skin of the dried organic binder is formed and when this is again wet, it forms clots. These clots are 20 objectionable since they are likely to drop off from the valve seat and fall on the engine and cause damage in subsequent operation.

I have discovered a composition which 25 overcomes all these objections and makes a bond free from organic material. This inorganic bond is preferably a finely divided mineral which is mixed with the abrasive grains and will form a smooth paste 30 with water.

I preferably employ for this purpose fuller's earth and especially that variety of this mineral known as "bentonite". Bentonite, when mixed with water, adsorbs the water 35 to a very large amount to form a gelatinous mass. Commercially, it is called "mineral gum", and it is this type of material which I preferably employ as the jelly-forming substance to carry the abrasive grains of 40 my abrasive composition.

In the preferred form of carrying out my invention, I first mix the mineral gum with about 6 parts of water to form a smooth paste, and then add the desired amount of 45 abrasive grains, which amount depends upon the purpose to which the grinding composition is to be put and also on the size of the abrasive particles. I also preferably add glycerine to give smoother consistency and

to retard evaporation. One formula I have employed with success is as follows:

|                 | Parts. |
|-----------------|--------|
| Mineral gum     | 8      |
| Silicon carbide | 40     |
| Water           | 49     |
| Glycerine       | 3      |
|                 | 55     |

However, I do not desire to limit myself to this formula nor to the use of glycerine nor to the use of silicon carbide as the 60 abrasive.

The advantages of this invention will be obvious to those skilled in the art, since there is no lubricant to interfere with the cutting actions of the particles and the material dries without a skin and forms no clots and may be readily made up again into a paste. Furthermore, my paste may be frozen without destroying its jelly-forming properties, whereas organic jellies when 70 frozen lose their jelly characteristics when again thawed out. These organic jellies, therefore, require an electrolyte, such as calcium chloride, to prevent freezing. This adds to the cost of the mixture and also 75 causes corrosion of the container before the paste is put into use. Such electrolytes are also likely to cause corrosion of the valve seats if not thoroughly wiped off after the grinding operation. A further advantage of 80 my composition is that it may be mixed with cold water since no heat is required at any stage of the manufacture; whereas in the former types, heat was required to form a smooth paste.

Changes may be made in the abrasive and the inorganic material used, the formula employed, the proportions used, etc., without departing from my invention.

I claim:

1. A paste for metal grinding formed with an inorganic material having a high absorptive power and having a granulated abrasive material incorporated therein, said paste also containing glycerine and being 95 free of silicate of soda.

2. As a new composition of matter, a grinding composition containing 8 parts of

bentonite, 40 parts of silicon carbide, 49 parts of water, and 3 parts of glycerine.

3. A paste for metal grinding comprising bentonite and water and having a granulated abrasive material mixed therein and a substance in the paste for lowering the freezing point of the water.

4. A paste for metal grinding formed with an inorganic material having a high

absorptive power and having granulated 10 abrasive material incorporated therein, said paste also containing water and a material for retarding the evaporation of the water, the paste being free of silicate of soda.

In testimony whereof I have hereunto set 15 my hand.

HENRY R. POWER.